

# United States Patent [19]

Schuster et al.

[11] 4,144,141

[45] Mar. 13, 1979

[54] AMMONIA FREE PALLADIUM  
DEPOSITION USING AMINOACETIC ACID

[75] Inventors: Hans-Joachim Schuster; Klaus-Dieter  
Heppner, both of Berlin, Fed. Rep. of  
Germany

[73] Assignee: Siemens Aktiengesellschaft, Berlin &  
Munich, Fed. Rep. of Germany

[21] Appl. No.: 863,044

[22] Filed: Dec. 21, 1977

[30] Foreign Application Priority Data

Dec. 21, 1976 [DE] Fed. Rep. of Germany ..... 2657925

[51] Int. Cl.<sup>2</sup> ..... C25D 3/52

[52] U.S. Cl. ..... 204/47; 204/43 N

[58] Field of Search ..... 204/47, 43 N, 109, 123;  
106/1.24, 1.28

[56] References Cited

FOREIGN PATENT DOCUMENTS

2506467 8/1976 Fed. Rep. of Germany ..... 204/43 N

Primary Examiner—G. L. Kaplan  
Attorney, Agent, or Firm—Hill, Gross, Simpson, Van  
Santen, Steadman, Chiara & Simpson

[57] ABSTRACT

An aqueous bath for galvanic deposition of palladium or palladium alloys and a process for using involving the use of aminoacetic acid as the sole complexing agent for palladium or palladium alloys in ammonium free, alkaline aqueous media.

4 Claims, No Drawings

## AMMONIA FREE PALLADIUM DEPOSITION USING AMINOACETIC ACID

### BACKGROUND OF THE INVENTION

The field of this invention is galvanic deposition of palladium or palladium alloys using aqueous plating baths.

In electrical engineering, palladium coatings produced by galvanic deposition are used as favourably 10 priced alternatives for galvanic hard gold coatings on contact components, such as plug connectors, for example. For this application, the palladium coatings must have uniformly semi-bright to bright surfaces, and be sufficiently ductile and pore-free. The baths used for 15 galvanic deposition have to be of simple composition and easy to top up so as to ensure uniform quality in the coatings deposited.

Galvanic baths producing coatings which meet the 20 named conditions operate in the alkaline pH range, mostly at high temperature, and contain substantial quantities of ammonia which has to be present mainly to form the ammine complexes needed for deposition.

With these known baths, the constantly evaporating 25 ammonia causes considerable difficulties in controlling the pH value. Ammonia has to be added continuously in metered quantities for the optimum pH range to be maintainable. In addition, the unpleasant and annoying odor of the evaporating ammonia makes the use of a 30 ventilator means necessary. One further disadvantage is that, in the case of partial coating with palladium, basic material containing copper is corroded by the ammonia vapours, and the corrosion products can contaminate the bath, and thereby change the technological properties of the deposited coatings for the worse.

A known bath for galvanic deposition of palladium nickel alloys also contains aminoacetic acid, but here, through the addition of ammonia, an alkaline pH value is set at which the palladium is present as an ammine 40 complex and not as an aminoacetic acid complex (Isbekowa D. V., Kudra O. K., Tschelikidi V. V., USSR, Saschtschita Metallow, vol IX No. 1/73, pp 108-110).

### BRIEF SUMMARY OF THE INVENTION

More particularly, this invention is directed to the use 45 of aminoacetic acid as a sole complexing agent for palladium or palladium alloys in an ammonium (and ammonia) free aqueous alkaline plating bath, and to a process for achieving plating of palladium or palladium alloys involving the use of such a bath.

A primary object of the present invention is to provide 50 an aqueous, ammonia-free palladium containing bath for galvanic deposition of palladium or palladium alloys which allows a desired pH range to be maintained exactly and which can be operated without any ventilator.

Another object is to provide an improved technique 55 for plating palladium and palladium alloys without using ammonium-containing aqueous media.

### DETAILED DESCRIPTION

By the present invention, a galvanic deposition bath 60 contains palladium in the form of a diglycinate palladium (II) complex using aminoacetic acid as the sole complexing agent. Such a bath gives pore-free, ductile and bright palladium or palladium alloy coatings of constant quality and does not give rise to any difficulties

as regards the maintenance of a pH range found to be an optimum. No ventilator is required.

In the prior art, the use of aminoacetic acid as a sole complexing agent for the deposition of palladium or 65 palladium alloys from an ammonia-free aqueous solution was unknown.

An aqueous bath in accordance with the present invention contains a diglycinate palladium (II) complex representable by the formula:



A bath containing such complex can be produced by any convenient procedure. For example, one can precipitate out palladium as a hydroxide from an aqueous  $\text{PdCl}_2$  solution followed by dissolution of hydroxide in aminoacetic acid aqueous solution, or by reacting a dissolved water soluble palladium salt (such as with dissolved aminoacetic acid where the anionic residue is removed by conventional measures or is allowed to remain in the bath).

The bath can also additionally contain conducting salts, and buffer reagents, such as chlorides, phosphates, citrates, acetates, and the like. The bath can also contain complexing agents like ethylenediamine-tetraacetic acid or nitrilotriacetic acid for complexing non-palladium metallic impurities, surface-active substances, or the like. The respective quantities of such additives employed in any given bath of the invention is similar to that used in prior art ammonium containing palladium plating baths.

Preferably, the palladium concentration in a bath of this invention ranges from about 1 to 50 g/l and preferably the quantity of aminoacetic acid (based on total 35 weight of added acid) ranges from about 1 to 150 g/l in such a solution. Moreover, the bath is advantageously set to a pH value ranging from about 7 to 12. Preferably, the pH value is set with alkali metal hydroxide. The alkali metal hydroxide is preferably preliminary dissolved in water to make up a 5 to 20 weight percent solution (10% being presently preferred) and then added to the previously prepared palladium solution.

When palladium alloy coatings or platings are to be deposited from a bath of this invention, the alloying 45 metals, if such are being used, are preferably added in the form of water soluble salts. The quantity employed can extend, if desired, up to the respective solubility limits thereof in water.

Thus, a preferred palladium galvanic deposition bath 50 of this invention comprises an aqueous solution having dissolved therein a diglycinate palladium (II) complex represented by the formula:



said solution being further characterized by containing:

- (A) from about 1 to 50 grams per liter of dissolved palladium,
- (B) from about 1 to 150 grams per liter of total added aminoacetic acid, and
- (C) sufficient dissolved alkali metal hydroxide to produce a solution pH ranging from about 7 to 12.

Optionally such bath can contain additional dissolved metals which are to be alloyed with palladium in a given coating. Also optionally, additives, such as described earlier, can be included in such a bath.

Suitable substrates for palladium coating using the bath of this invention include metals such as copper,

iron (including steel), and like metals used as contact components in electrical devices, circuits, etc. Presently preferred palladium coatings produced by using a bath of this invention containing at least about 50 weight percent palladium on a 100 weight percent total coating weight basis. In any given instance a product coating composition can be determined by the selection of components contained in a bath of this invention.

### EMBODIMENTS

The present invention is further illustrated by reference to the following examples. Those skilled in the art will appreciate that other and further embodiments are obvious and within the spirit and scope of this invention from the teachings of these present examples taken with the accompanying specification. The quantities indicated for the individual components relate in each case to one liter of aqueous solution.

#### EXAMPLE 1

An aqueous solution having the following composition is prepared:

Pd in form of  $\text{Pd}(\text{CH}_2\text{NH}_2\text{COO})_2$ : 10 g/l

Aminoacetic acid: 50 g/l

Ethylenediaminetetraacetic acid: 5 g/l

To the resulting solution is added sufficient 10% aqueous solution of potassium hydroxide to produce a product solution having a pH of 9 while maintaining a solution temperature of 60° C.

When a current density of 1.0 A/dm<sup>2</sup> is applied across a bath comprised of such product solution, it is found that the bath gives a bright, abrasion-resistant palladium coating on a clean copper substrate surface. The current yield is 100%.

#### EXAMPLE 2

An aqueous solution having the following composition is prepared:

Pd in the form of  $\text{Pd}(\text{CH}_3\text{COO})_2$ : 8 g/l

Aminoacetic acid: 20 g/l

Potassium dihydrogen phosphate: 50 g/l

Nitrilotriacetic acid: 10 g/l

To the resulting solution is added sufficient 10% aqueous solution of potassium hydroxide to produce a product solution having a pH of 8 while maintaining a solution temperature of 25° C.

When a current density of 0.2 A/dm<sup>2</sup> is applied across a bath comprised of such product solution the bath gives a bright, pore-free coating on a clean copper substrate surface. Coating hardness equals 230 kp/mm<sup>2</sup>.

#### EXAMPLE 3

An aqueous solution having the following composition is prepared:

Pd in the form of  $\text{PdCl}_2$ : 20 g/l

Ni in the form of  $\text{NiSO}_4 \cdot 6\text{H}_2\text{O}$ : 20 g/l

Aminoacetic acid: 100 g/l

Sodium chloride: 50 g/l

To the resulting solution is added sufficient 10% aqueous solution of sodium hydroxide to produce a product solution having a pH of 8 while maintaining a solution temperature of 45° C.

When a current density of 0.5 A/dm<sup>2</sup> is applied across a bath comprised of such product solution, the bath gives a hard, abrasion-resistant palladium nickel alloy coating on a clean copper substrate surface.

### EXAMPLE 4

An aqueous solution having the following composition is prepared:

Pd in the form of  $\text{Pd}(\text{CH}_2\text{NH}_2\text{COO})_2$ : 5 g/l

Ag in the form of  $\text{Ag}_2\text{SO}_4$ : 10 g/l

Aminoacetic acid: 100 g/l

To the resulting solution is added sufficient 10% aqueous solution of sodium hydroxide to produce a product solution having a pH of 10 while maintaining a solution temperature of 50° C.

When a current density of 0.4 A/dm<sup>2</sup> is applied across a bath comprised of such product solution, the bath gives a smooth, pore-free palladium-silver coating on a clean copper substrate surface.

As is apparent from the foregoing specification, the present invention is susceptible of being embodied with various alterations and modifications which may differ particularly from those that have been described in the preceding specification and description. For this reason, it is to be fully understood that all of the foregoing is intended to be merely illustrative and is not to be construed or interpreted as being restrictive or otherwise limiting of the present invention, excepting as it is set forth in the hereto appended claims.

I claim:

1. An aqueous ammonia-free bath for galvanic deposition of palladium metal containing palladium in the form of a diglycinate palladium II complex and aminoacetic acid as complexing agent, said bath being further characterized by containing:

(A) from about 1 to 50 grams per liter of dissolved palladium,

(B) from about 1 to 150 grams per liter of total added aminoacetic acid, and

(C) sufficient dissolved alkali metal hydroxide to produce a solution pH ranging from about 7 to 12.

2. The bath of claim 1 wherein said alkali metal hydroxide is potassium hydroxide.

3. The bath of claim 1 wherein said alkali metal hydroxide is sodium hydroxide.

4. The bath of claim 1 wherein said diglycinate palladium II complex is represented by the formula  $\text{Pd}(\text{OOCCH}_2\text{NH}_2)_2$ .

\* \* \* \* \*